

Jan. 5, 1937.

C. F. SCHMIDT, JR., ET AL

2,067,066

COATED MATERIAL

Filed June 19, 1933



Fig. I

Fig. II



Fig. III



Fig. IV



Fig. V

INVENTOR  
Clifton F. Schmidt  
and  
George L. Ball  
by Christy, Christy and Wharton  
attorneys

## UNITED STATES PATENT OFFICE

2,067,066

## COATED MATERIAL

Clifton F. Schmidt, Jr., and George L. Ball,  
Pittsburgh, Pa.

Application June 19, 1933, Serial No. 676,540

2 Claims. (Cl. 215—37)

This invention relates to a fibrous or pulpous flexible and compressible material, so coated as to preserve its flexibility and compressibility, while supplying the material with a sealing coating, which is tough and flexible, and which is insoluble and chemically neutral.

A further object of the invention is to provide a material coated in this manner which may be economically manufactured, so that together with its other characteristics it is eminently suited to use as a liner for bottle caps and other closures applied to containers for foods, beverages, cosmetics, and various chemicals and other materials.

We have found that if a sealing coat having a resoleate base be applied directly to a porous absorbent material, such as pulp or fiber board, the coating material so saturates the board as to cause waste of the coating material and to impair the flexibility and compressibility of the board. Such board is therefore unsuitable as a liner for bottle caps and similar closures, in that it does not conform to the edge of the neck or other opening of the container, by compression, to provide a tight seal in the closure. We have further discovered that a compressible absorbent material coated with a colloidal material alone is not wholly suitable for such purposes. Such material is thermoplastic, thus tending to cement a closure to a container. It is of such nature that it may be affected by certain foods, beverages, cosmetics, and so forth, which are usually put up in containers to which a lined closure may be applied.

We have discovered that we may render a compressible absorbent material, such as pulp or fiber-board generally suitable for use in making liners for bottle caps, and for similar uses, by first applying to a surface of the material a stop coat or coats of a suitable colloidal coating material; and by applying to the underlying coat an overlying coating of a suitable resoleate base coating material. This outer coating gives the material a flexible, elastic and wholly coherent outer skin or covering, which is in itself neutral, and which is highly resistant to acids, fumes, salts, and products of fermentation.

For application it is necessary that the colloidal material be prepared with suitable evaporative solvents, and that the coating composition comprising it contains a sufficient percentage of the solid ingredient to deposit a substantial film on a surface to which the coating composition is applied.

We have discovered that an inexpensive and particularly desirable colloidal coating fluid may

be made by suitably dissolving photographic film, which when used and discarded is a waste material. The photographic film used by us contains in its composition nitro-cellulose and various plasticizers. By the term "photographic film," as used throughout the specification and claims, we therefore intend to designate "nitro-cellulose film," which is the photographic film in most common use, and not cellulose acetate film.

The difficulty which has been experienced in the application of a solution of photographic film to a surface is due to the fictitious viscosity or apparent body of the film material in solution. That is, when a coating material comprising photographic film, dissolved in the solvents previously used, is applied to a surface, such a small quantity of the solid ingredient has been dissolved initially, and deposited on the surface, that an adequate film is not formed. In order that an adequate quantity of material be deposited on a surface to form a substantial film, it is necessary that there be a sufficient quantity of the film-forming solid in any given volume of solvent.

We have discovered that we can obtain a flowable coating material of honest body by producing a base solution of photographic film in acetone as the sole solvent for the photographic film. We have found that if acetone, without substantial admixture of other solvents, be used, we can dissolve more than two pounds of scrap photographic film in each gallon of acetone. In this solvent, used alone, the scrap photographic film loses its tendency toward fictitious viscosity, and an adequate quantity can be dissolved to form a flowable coating material of honest body, capable of depositing a dense, continuous film of adequate depth.

We therefore make up our base solution by dissolving in acetone as great content of scrap photographic film as the acetone will receive under normal production conditions. This content is in excess of two pounds of scrap photographic film per gallon of acetone, and the solution thus made up is readily flowable, in spite of its high content of solid matter. Since the matter of "body" is of prime importance in securing a deep, dense, and uniform film, we prefer to use our base solution, either alone or mixed with other film-forming materials, without the addition of any substantial quantity of thinning fluids.

In order that a coating material of great elasticity may be produced, utilizing our base solution, we may mix it with a processed oil, which has, in admixture, the quality of producing films

5

15

20

25

30

35

40

45

50

55

of great elasticity. Such oil may be one of the highly refined, highly oxidized, aerated, linseed oils, which are in general use, and which fall within the loose trade designation of "blown" 5 oils. A preferred oil for admixture, however, is the processed linseed oil sold by Archer-Daniels-Midland Company under the name "A. D. M. 100" oil.

The oil known by the trade name of "A. D. M. 10 100" oil is a drying oil, preferably linseed oil, which has been oxidized, at temperatures relatively so low as to prevent undue polymerization, and which has undergone under these low temperature conditions oxidation sufficient to render 15 the oil soluble in ethyl alcohol. The oil as used is in the form of a solution in about 15% of ethyl alcohol.

For the reasons explained in our co-pending 20 application, Serial No. 676,527, filed June 19, 1933, the "blown" oil of common production may be commingled with the base solution in a quantity 25 by weight of from one-fifth the weight of the photographic film content up to the weight of the photographic film content. The "A. D. M. 100" oil we may mix with the base solution in a 30 weight of from equality with the weight of the photographic film content up to four times the weight of the photographic film content. Both the highly oxidized highly refined "blown" oil of 35 common production, and the specialized processed linseed oil known as "A. D. M. 100" oil are film-forming materials, and the latter has the quality of entering wholly into film formation to provide an extraordinary toughening and plasticizing effect in the film as a whole.

For our present purpose, that is, the formation 40 of a stop coat on absorbent material, such as news board or the like, which is to be cut into liners for closure caps, or into gaskets and the like, we prefer to use the "A. D. M. 100" oil in relatively great quantity with respect to the photographic film content of the base solution. We have found a two-to-one mixture of "A. D. M. 100" oil with the base solution thoroughly satisfactory 45 for use as a stop coat in the coating of news board for use as closure cap liners.

If our coating material could in all instances be applied under ideal conditions, it might be used, either alone or in combination with an oil 50 capable of elastic film formation, without the addition of any other ingredient, or ingredients. It is, however, a fact that the base solution has a relatively high "dew point," and tends to "blush" when applied under any but perfect atmospheric 55 conditions. We therefore add a relatively small quantity of a regulatory fluid, which is desirably pine oil, butyl lactate, or a mixture of these fluids.

A preferred regulatory fluid is the mixture of 60 pine oil and butyl lactate, in the proportion of 2 parts of pine oil to 1 part of butyl lactate. This we desirably add to the base solution, or to the mixture of base solution and processed oil, in a quantity of from 10 to 14 ounces of regulatory 65 fluid to each gallon of base solution, or 5 to 10 ounces of regulatory fluid to a mixture of base solution and processed oil.

As a substitute for the butyl lactate, as a regulatory fluid, we may use hexalin, methyl hexalin, 70 or butyl "cellosolve" which is the monobutyl ether of ethylene glycol. As a substitute for pine oil, we may use dipentene, a fluid having a body midway between that of pine oil and that of wood turpentine.

75 The regulatory fluid serves as a general cor-

rective, present in the coating material, for atmospheric conditions which might otherwise be unfavorable, by lowering the "dew point" of the coating material, and preventing "blushing" in the film formed from the coating material. 5

The coating material may be applied to a surface which is to be covered by wiping, brushing, spraying, or by rolling the material on the surface. It also may be used as a dip coating. Our preferred manner of application is to place an 10 excess of the coating material on a surface to be coated, and to spread it evenly thereon, removing surplus material, by use of a "doctor knife," or other suitable scraper. This mode of application is particularly desirable for applying the 15 coating material to a pulp or fibre board, such as news board, for the reason that the nap of the base material is smoothed down as the coating material is applied.

After application, the coating is subjected de- 20 sirable to forced evaporation, at such moderate temperature, not in excess of 300° Fahrenheit, as will not tend to injure the film formed by evaporation, or the material on which the coating material has been spread.

It is an advantage of our coating material that it anchors firmly to the surface of an absorbent material, such as a pulpy or fibrous board, or to the surface of a closely woven fabric such as 30 canvas, without penetrating the body of the material coated to any appreciable extent.

In the accompanying drawing, Figure I illustrates on a greatly enlarged scale a section of pulp or fiber board with our stop coat spread thereon; Figure II is a similar view, but showing 35 the material with a resistant coat also applied over the colloidal stop coat and forming a wholly coherent film thereon; Figure III is a cross-sectional view through a bottle cap and liner on a greatly enlarged scale, the liner being composed 40 of our specially coated board; Figure IV is a cross-sectional view through the same bottle cap, showing the compression of the liner attendant upon use of the cap as a closure for a bottle; and Figure V is a cross-sectional view through a similar 45 bottle cap, illustrating the use of a lining board which has received a colloidal coating on both of its surfaces.

Referring to Figure I of the drawing, the intermediate product as shown therein, and as described above, comprises the pulp or fiberboard proper, designated by reference numeral 1. Reference numeral 2 designates the colloidal stop coat remaining after evaporation of the solvents. It will be noted that this stop coat 2 does not 55 penetrate deeply into the board 1, although it is anchored to it.

The board, with the stop coat 2 dried thereon, is then in condition for a resistant, or contact, 60 coat designated by reference numeral 3 in Figure II, and succeeding figures of the drawing. This outer contact coat may be any suitable coating material providing when dry an elastic film which is wholly continuous, which is of itself neutral, and which is resistant to the action of acids, 65 salts, alkaline materials, and the products of fermentation. While various coating materials, such as waxes and various synthetic resin base coatings, fulfill these requirements in greater or lesser degree, we have found by experiment that 70 a peculiarly satisfactory outer coating is obtained by reducing a resin of the modified ester gum and oil type to a varnishlike consistency with suitable quantities of petroleum, pine oil and coal tar distillate. This coating we apply in any suitable and 75

expeditious manner on the board previously provided with a stop coat 2, and subject the board so coated to baking.

It will be observed in Figure II of the drawing 5 that this outer, or contact coating has not penetrated the underlying board to stiffen the board or otherwise detract from its flexibility and compressibility. It will be noted further, from this figure of the drawing, that the outer, or contact 10 coating serves to fill any minute apertures which may be present in the stop coat. Such minute apertures are of very rare occurrence with the preferred coating material hereinbefore disclosed, for the reason that it is formed specifically to provide a dense coating, of uniform depth, and without "pin holes" or other weakness.

Figure III of the drawing shows the use of our prepared board as a liner in a suitable crimped metallic shell 4, the shell and liner constituting a 15 sealing and impervious bottle cap.

Figure IV of the drawing illustrates the manner in which both the board itself and the elastic coating thereon seals against the mouth 5 of a bottle or the like. It is to be observed in this 20 figure that the board proper 1 has been compressed, and that both the inner and outer coatings 2 and 3 have stretched sufficiently in accordance with the compression of the board to prevent any cracking or scaling of the coating. The liner coated in accordance with our practice 25 therefore provides a tight and efficient seal, which is wholly impervious and which is not attacked by the contents of the vessel to which the closure member has been applied.

In Figure V of the drawing, a colloidal coating 30 has been applied to both faces of the board. In this instance the coating 6, which lies against the inner surface of the bottle cap 4, serves to cement the liner in the shell if it be heated, or provided 35 with a drop of solvent, and pressed firmly into the shell.

We have referred above to the fact that we 40 prefer a finishing coat of special coating material produced by reducing a resin of the modified ester gum and oil type to a varnish-like consistency. Coating materials of this type may be 45 made up of various initial ingredients and according to various methods of manufacture; but all may properly be described as "resoleate base" 50 materials, involving as they do the heat treatment of a modified ester gum with a suitable oil. We may, however, give a typical example of the procedure in making up the resoleate base for such coating material.

The starting material is a modified ester gum, and we have found satisfactory the modified gum 55 known as Lewisol No. 2, and widely sold under that name by John T. Lewis, of Providence, Rhode Island. While the exact composition of this resin 60 is a trade secret, a resin may be made having qualities sufficiently like that of Lewisol No. 2 to be satisfactory for our purpose by esterizing rosin, and fusing the esterized rosin with a fatty acid, such as the fatty acid of linseed oil or 65 China-wood oil.

The modified ester gum may then be worked 70 up into a resoleate base by the following procedure. Assuming that Lewisol No. 2 is the modified ester gum used, it is heated to 525° F. with a portion of China-wood oil. When this temperature is reached, it is checked with a part of the 75 total quantity of China-wood oil, and when the temperature of 525° F. is again reached, it is checked with the balance of the China-wood oil. The gum and China-wood oil is again brought to

525° F., and an alkali-refined linseed oil, cooked to give heavy body, is added. The batch is held at a temperature of 525° F. for a period of about one hour, to give body, is cooled, and reduced. The quantity of China-wood oil and linseed oil 5 may be varied in accordance with the desired elasticity of the resulting products, but the total quantity of oil should desirably lie within the range of 20 to 40 gallons for each 100 pounds of resin. The resulting product is a viscous resole- 10 ate material.

Instead of Lewisol No. 2, as the starting resin, we may use Amberol No. 801, widely sold under that designation by Resinous Products and Chemical Company, Inc., of Philadelphia, Pennsylvania; or we may use Beckacite No. 1112, widely 15 sold under that designation by Beck, Koller and Company, Inc., of Detroit, Michigan.

This outer, or contact, coat as so formed is 20 clear, transparent, is free from after-yellowing, and provides a good vehicle for pigment, if a colored product is desired. The coated material, after application of the contact coat, should be heat treated at a temperature not in excess of 300° F., in order that it may not injure inflammable 25 material, to which the two diverse coatings have been applied. The heat treatment should be conducted for a substantial period, as from thirty to sixty minutes, in order to convert the outer coating material to insolubility and 30 complete neutrality.

As so treated, the coating material is odorless, tasteless, sterile, is highly resistant to the action of acids and alkalis, and presents unusual resistance to the action of alcohol. The coated material as a whole is so highly impenetrable that it may be considered wholly impenetrable by water, food juices, and substantially all liquids which occur with food products, toilet preparations, or the like, which are sold in capped containers. These qualities render the use of an inexpensive, compressible material such as news 40 board, when coated as described, peculiarly suitable for use in making liners for bottle caps, jar covers, and the like. In addition, the elasticity 45 of both the stop coat and the outer, or contact, coat serves to produce a close, impervious seal with the edge of a bottle neck, jar, or the like.

One result of the forced evaporation to which the stop coat is subjected, and the heat treatment to which the contact coat is subjected, is to so dry the news board, or other similar material, that it becomes too dry to be readily punched or stamped into shaped pieces, such as the circular pieces used as liners for closure caps. 55 For this reason, the material, after heat treatment, is desirably treated in a humidifier. As the sterility of the material would be impaired by such moistening, it would not be then so suitable for use as lining material in the closure 60 caps of food and beverage containers. To avoid loss of sterility, when the coated material is to be used for such purpose, we use in the humidifier a dilute germicidal solution. We have found that a water solution of resorcin of germicidal 65 strength, or a dilute benzoate of soda solution gives the desired moistening, while preserving the sterility of the material, and without giving an odor to the material.

Considering our coated material solely as a 70 liner for bottle caps, it possesses the distinction of being a single piece liner, while furnishing an elastic and wholly impervious sealing medium. It thus differs widely from bottle cap liners which comprise a base of cork composition, or cork sub- 75

stitute, with a piece of paper, waxed or otherwise treated, adhesively attached thereto.

Because our material, considered as a closure cap liner, is a single piece article, it may be manufactured with an economy in manufacturing steps or operations. That is the news board, or its substantial equivalent, may be coated in continuous lengths, and made into single piece closure cap liners merely by a machine punching,

10 without any finishing treatment.

It should be understood that where the word "coat" is used throughout the specification and claims, it should be held to describe a coating formed by more than one application of coating

15 material, as well as a coating formed by one application alone.

This is a continuation in part of our previously filed application, Serial No. 624,044, filed July 22, 1932, for an improvement in Coated material.

We claim as our invention:

1. A single piece liner for use in container cap closures composite of an absorbent and compressible fibrous or pulpous board base and a double coating of diverse layers covering one face of said absorbent and compressible base; the said coating comprising an elastic primarily clear and non-penetrating stop coat of nitrocellulose film

together with an oxidized alcohol-soluble and alcohol-containing linseed oil of but slight polymerization forming a stop coat anchored to the absorbent base, and an elastic impermeable contact coat of coating material comprising a modified ester gum and oil resin heat cured to a condition of relative insolubility overlying the said stop coat and separated from the absorbent and compressible base thereby.

2. A single piece liner for use in container cap closures composite of an absorbent and compressible fibrous board base and a double coating of diverse layers covering one face of said absorbent and compressible base, the said coating comprising an elastic primarily clear and non-penetrating stop coat of nitrocellulose photographic film together with an oxidized alcohol-soluble and alcohol-containing linseed oil of but slight polymerization forming a stop coat anchored to the absorbent base, and an elastic impermeable contact coat of coating material comprising a modified ester gum and oil resin heat cured to a condition of relative insolubility overlying the said stop coat and separated from the absorbent and compressible base thereby.

CLIFTON F. SCHMIDT, JR.  
GEORGE L. BALL.